

## UNITED STATES PATENT OFFICE

2,093,651

## DYEING FIBROUS MATERIALS

Gustave A. Widmer, Philadelphia, Pa., and Edward W. Pierce, Clifton, N. J.

No Drawing. Application February 9, 1933,  
Serial No. 656,024

14 Claims. (Cl. 8—5)

It has been proposed to impregnate cotton or rayon fabrics with diluted aqueous solutions of urea-formaldehyde condensation products with the purpose of producing an anti-crease effect after suitable curing and processing.

It has been found that carbamide-formaldehyde compounds if properly processed, produce unexpected and useful results in the dyeing art, and this application is a description of the new processes and products developed by using such compounds as a fixing agent for dyestuffs and pigments.

These processes can be classed into two groups, both of which however cover fixing coloring matters, but the first group comprises processes in which acid dyes, wool or silk dyes, and the like are used which possess a chemical affinity for heat-treated carbamide-formaldehyde compounds and wherein the dye is therefore chemically affixed. The second group comprises processes using pigments, metal powders or finely divided insoluble dyes, the carbamide-formaldehyde compounds acting as an insoluble binder, affixing these pigments mechanically. Combinations of the processes taken from both groups respectively are possible.

All these processes have one common feature: an aqueous or aqueous-alcoholic solution of a carbamide-formaldehyde compound is used for impregnating the fibrous material to be dyed, and thereafter the material is dried, usually at a moderate temperature. Then the soluble carbamide-formaldehyde compound which is deposited during the drying operation, in, on and around the fibres is converted into its insoluble form by applying a suitable heat treatment. This insoluble form is the final form of the product and possesses surprising properties.

The insoluble carbamide-formaldehyde product is found to have a decided affinity for acid dyes as they are usually used for dyeing wool or silk, i. e., animal fibres. In other words: after properly processing a fibrous material, for instance cotton fabric, with a carbamide-formaldehyde compound and thereafter transforming it into its insoluble form it can be dyed with the same dyes as wool or silk. This fact offers great possibilities because, in many cases the wool dyes are considerably cheaper and light-faster than direct cotton dyes, and in other cases a brilliancy of shade is obtainable not to be produced with direct cotton dyes.

Many modifications of this process can be used in order to bring about this same result, by subsequent or simultaneous impregnation of fibrous

material with carbamide-formaldehyde compounds and dyeing or printing, applying reserves or intensifiers, as indicated in the examples given below, which examples will serve to demonstrate some of the many feasible ways of practicing the invention.

As materials to be impregnated, all kinds of cellulosic fibrous material can be used,—cotton, rayon, linen, jute, ramie, etc., in form of sheets (fabrics or paper), spun in form of yarn, or loose fibre. Most practical however is the sheet form where a continuous process can be used to bring about the impregnation by immersion, dipping, brushing, printing, spraying, etc.

The impregnation step may be carried out by a simple dipping and squeezing operation, leaving in the fabric or other fibrous material the desired amount of carbamide-formaldehyde compound. If the bath contains at the same time, an acid dye, the dye is chemically affixed by the carbamide-formaldehyde compound by heat-treating the material afterwards and thereby making it insoluble in water and solvents. If the impregnation is done with the soluble carbamide-formaldehyde compound, it may be heat-treated and then dyed subsequently in the usual manner with an acid dye, or it may be printed in various ways.

"Reserves" may be printed on, for example in organic bases like sodium hydroxide, barium hydroxide, etc. These substances prevent the proper reaction from taking place during the heat treatment of impregnated material, so that upon subsequent dyeing the printed places show no affinity for the acid dye and therefore remain white or nearly so.

Instead of "reserves", "intensifiers" may be printed on the impregnated material. Organic bases of the type of methylamine, ethylene diamine, etc., may be used for this purpose. Very surprising is also that hexamethylenetetramine and other ammonium compounds, like ammonium acetate act as "intensifiers", whereas free ammonia acts as a "reserve." By the use of some of these "intensifiers" the strength of the color is greatly enhanced, much stronger than without them, due to increased selective affinity for acid dyes.

Simultaneously with "intensifiers" or "reserves" other suitable dyestuffs may be printed on impregnated material and thereby by proper processing multicolor effects be produced.

The heat treatment of the impregnated fibrous material which converts the carbamide-formaldehyde compound from the soluble into the insoluble form may be applied in different ways. The ma-

terial may for instance be steamed after impregnation in the steaming equipment commercially used in dyeing plants, where it is heated in presence of steam at temperatures over 100 degrees C. under pressure. Or the material may if it is in sheet form, be subjected to the influence of dry heat, bringing it into contact with a hot plate heated to 130 to 170 degrees C., or carrying it slowly in a continuous way over the surface of a hot roll or a steam cylinder heated to about the above-mentioned temperatures.

The carbamide-formaldehyde compounds are transformed into their insoluble form according to their properties under somewhat different conditions. Dimethylolurea, mixtures of mono- and dimethylolurea, or mono-methylolurea as well as their more advanced condensation stages have been found to require for instance two minutes at 165 degrees C. or 20 minutes at 130 degrees C., in order to secure good results, that is, to assure that the greatest part of the compound remains in the fibrous material after boiling with a diluted soap solution.

Mixtures of methylolurea and methylolthiourea, or their more advanced condensation stages, have been found to require a somewhat shorter heat treatment, especially if there is not too much methylolthiourea compound present.

The heat treatment may be carried out in acid, neutral, or basic solution. Advantageously organic acids are used as for instance, acetic acid, formic acid, tartaric acid or the like. If the use of inorganic acid is contemplated, very weak acids should be taken as for instance carbonic acid or boric acid, because of the detrimental effect of the strong inorganic acids to cellulose when heated. (Carbonizing effect.)

It has been found that the heat treatment in perfectly neutral solutions requires a slightly longer time, but produces the same results as the heat treatment in acid solution.

The heat treatment in basic solution produces results, which are not normal, as indicated above. In presence of inorganic bases like sodium hydroxide etc., the carbamide-formaldehyde products do not get insoluble and subsequent soaping removes them: They act as "reserves." In presence of organic bases like ethylene diamine, etc., the heat treatment produces an increased affinity for acid dyes; they act as "intensifiers."

The desirable characteristics are obtained at their maximum when the amount of insoluble carbamide-formaldehyde compound is about ten to thirty per cent of the weight of the fibrous material. Under ten per cent the desirable properties disappear slowly, and over thirty per cent the material gets increasingly harsher and eventually stiffer. But in presence of the proper amount the material is not of decreased textile value but rather shows improved textile characteristics.

Instead of carbamide-formaldehyde products in their narrower sense, namely, urea-formaldehyde products, also the corresponding formaldehyde products of substituted ureas, like methylurea, phenylurea, dicyan-diamide, biuret, etc., or urea homologues like thiourea or guanidine may be used, or mixtures thereof. Mixtures of some urea, biuret, guanidine, cyanuric acid etc., obtained by decomposing urea by heat at about 160° C., are also very suitable.

While some of the above substances operate very well in their pure form, and even show increased affinity for acid dyes, like for example, thiourea-formaldehyde compounds, dicyan-

diamide formaldehyde compounds, formaldehyde compounds of heat-treated urea, etc., they very often enhance also the desirable characteristics of the final product, when used in admixture with urea-formaldehyde products. This is particularly so with thiourea and dicyan-diamide.

Thiourea is particularly interesting due to the very greatly increased affinity it imparts to the cellulosic material. But dicyan-diamide, guanidine and heat-treated urea also produce markedly increased affinity for acid dyes in comparison to urea compounds alone.

The processes indicated above are as a matter of course capable of an infinite number of variations according to the composition of impregnating material, the material, the dyestuff, or the method of dyeing, etc. This same applies to the processes disclosed below in which primarily the mechanical fixing property of such carbamide-formaldehyde compounds is contemplated.

It has been found that carbamide-formaldehyde compounds in their soluble stage are easily incorporated in mixtures containing pigments, such as ultramarine, carbon black, etc., or metal powders like aluminum powder. In a similar manner it is easy to incorporate organic color pigments, color lakes, water insoluble dyes, as for instance nigrosine (spirit soluble), aniline black, oxidized vat dyes (like indigo), and other finely divided insoluble coloring matter. After preparing such mixtures with carbamide-formaldehyde compounds, advantageously in form of suspensions or pastes,—fibrous materials are treated therewith by an impregnation or printing operation. After subsequent drying and heat-treating, the finely divided coloring matter is firmly affixed to the treated fibres, because the color particles are imbedded in the colorless insoluble carbamide-formaldehyde compound acting as a binder. Wash-fast dyeings and printings with pigments of highest light resistance can thereby be cheaply produced,—a result heretofore impossible.

This process relating to mechanical affixing of finely divided coloring matter may be applied to all kinds of fibrous materials, not only cellulose but also wool or silk. The process is particularly adaptable to such materials in sheet form, which allows easy impregnation by immersion, dipping, brushing, printing, spraying, etc. The material in such form namely as a fabric or paper, can then be processed in a continuous way. Such paper has for instance use for wall paper and the like, due to its wash and light fastness.

As a matter of course "reserves" can also be applied in this process which result in washing the insoluble coloring matter out after heat-treatment by hot soaping, leaving white places.

It is evident from the foregoing general discussion, as well as from the several specific examples hereinafter set forth, that the present invention is by no means limited to the urea-formaldehyde condensation product, but that it envisages condensation products of formaldehyde and derivatives and/or homologues of urea, such as methyl urea, biuret, phenyl urea, dicyan-diamide, biuret, guanylurea, thiourea, guanidine, etc.

The following examples illustrate some of the many ways of carrying out the invention.

#### Example 1

An impregnation solution is made up as follows: 30 gm. of dry dimethylolurea are dissolved in 150 cc. warm water and the solution brought up to 75

200 cc., i. e., 15% strength. The pH value is adjusted to pH=4.5 by adding acetic acid and cotton cloth is immersed therein for a few minutes. The cloth is squeezed out to 100% expression (i. e., the weight of the wet impregnated cloth is 5 100% more than the original dry cloth). Then it is air-dried and heat-treated by ironing with a hot iron for 2 minutes. The cloth is now cut into suitable pieces for dyeing.

10 (a) 20 cc. of a 1/4% solution of Kiton fast yellow 3G (Color Index 645) is diluted to 200 cc. then 1 cc. of formic acid is added and the temperature raised to 130° F. A piece of the above treated cotton fabric is dyed in this bath for 20 minutes, rinsed in water and dried. The resultant color is a medium strong yellow, whereas the 15 untreated, unimpregnated sample, dyed under the same conditions is almost white.

Exactly in an analogous manner further samples of the impregnated heat-treated cotton fabric are dyed with

(b) Alizarine Sapphire Blue GS

(c) Kiton Fast Red 4 BL (C. I. Sup. Pg. 44).

The results of b and c are analogous to Example 25 a.

(d) Alizarine Sapphire Blue GS is dyed on a crepe-rayon fabric which was previously treated as the cotton cloth. It is dyed a blue of medium strength whereas the untreated rayon sample 30 dyes a very light tint.

#### Example 2

(a) A sample of cotton cloth impregnated as described in Example 1 is, before heat-treating it, 35 printed with a printing paste containing 95% British gum (the commercially available printing paste, consisting of cooked starch) and 5% ethylene diamine. The print is then air-dried and heat-treated by hot ironing for 2 minutes.

40 A dyestuff solution is now made up as follows: 20 cc. of a 1/4% solution of Alizarine Sapphire Blue GS are diluted to 200 cc. and 1 cc. of formic acid added. The printed and heat-treated cloth is now dyed for 3/4 of an hour at 120-130° F. 45 rinsed and dried.

Very surprisingly the printed places appear in a deep blue shade, indicating that ethylene diamine intensifies the affinity of the carbamide compound for this acid dye, and does not act as 50 a reserve, as expected. A sample of this printed cloth was exposed 42 hours to the influence of artificial sunlight in the Atlas Fadeometer. The light bluish tinted ground faded somewhat and the heavy blue design remained practically unchanged. This shows that the general light fastness of this wool dyestuff is retained if used on 55 cotton according to this process.

(b) In an analogous manner as in Example 2a impregnated cotton cloth is printed with a 60 paste containing 2% NaOH in British gum. Then it is heat-treated and dyed as described in 2a. The sample dyes in the unprinted places a medium blue, and in the printed places a very faint blue tint. It appears therefore, that the 65 caustic acts as a reserve.

#### Example 3

Cotton fabric samples are immersed in the following solutions:

70 (a) 25% solution of dimethylolurea  
(b) 25% solution of an equimolecular mixture  
of mono- and dimethylolurea  
(c) 25% solution of monomethylolurea  
(d) Water.

75 The samples are then expressed to 100% (dou-

ble weight), and after air-drying heat-treated on a hot plate between paper layers 3 minutes at about 320° F. Then each sample is dyed separately in a bath containing 20 cc. of 1/4% Alizarine Sapphire Blue GS in 200 cc. water plus 1 cc. 5 formic acid, 3/4 of an hour at 130° F. Then rinsed and dried.

Sample d (blank sample) is dyed a very faint tint of blue, samples c, b and a are increasingly deeper blue,—sample a impregnated with di- 10 methylolurea is the strongest blue.

None of these solutions have been acidified, which insures better stability of the methylolurea solutions. They remain clear and stable for a much longer time than the acidified solutions of 15 methylolurea, which latter become turbid after about 1/4 of an hour.

#### Example 4

To 100 cc. of a 15% solution of dimethylolurea 20 there is added 25 cc. of a 1/4% solution of Alizarine Sapphire Blue. A sample of cotton cloth is immersed therein and after air-drying, heat-treated for 2 minutes on a hot plate at about 320° F. It is then soaped in hot 1% soap solution and shows 25 after rinsing and drying a medium blue of very good wash fastness.

#### Example 5

A printing paste is prepared as follows: 30

|                                 | Grams   |
|---------------------------------|---------|
| Alizarine Sapphire Blue GS..... | 2       |
| Tartaric acid .....             | 1       |
| Dimethylolurea dry .....        | 12.5    |
| Water.....                      | 36 35   |
| British gum.....                | 48.5    |
| <br>Total.....                  | <br>100 |

With this paste a plain cotton cloth is printed, 40 air-dried and steamed for 1/2 hour at 12 pounds per square inch steam pressure in a laboratory steambox.

On soaping a portion of the sample in 1% soap solution at about 170° F. it bleeds somewhat, 45 which shows that the heat treatment is not quite sufficient.

Therefore another portion of the steam-treated sample is further heated 2 minutes at 320° F. A soaping test of this sample shows not a trace of 50 bleeding which indicates that the heat treatment was complete. A sample treated as last described was exposed in the Atlas Fadeometer 42 hours to the influence of artificial sunlight. It does not show any fading. This indicates that the light- 55 fastness of this dye is here on cotton just as good as if the dyestuff was used on wool.

#### Example 6

The following printing paste is prepared: 60

|                                                                                | Grams      |
|--------------------------------------------------------------------------------|------------|
| Cibanone Violet 4B (Micro-powder, water-<br>insoluble, acts as a pigment)..... | 2          |
| Tartaric acid .....                                                            | 1          |
| Dimethylolurea .....                                                           | 12.5 65    |
| Water.....                                                                     | 36         |
| British gum.....                                                               | 48.5       |
| <br>Total.....                                                                 | <br>100 70 |

A cotton fabric is printed with the above paste, air-dried, and then heat-treated on a hot plate 2 minutes at 320° F. The soaping test shows no bleeding, which indicates that the pigment is 75 firmly, mechanically affixed to the fibre.

**Example 7**

A printing paste is prepared as follows:

|                  | Grams |
|------------------|-------|
| Lampblack        | 4     |
| 5 Dimethylolurea | 15    |
| Water            | 38    |
| British gum      | 43    |
| Total            | 100   |

10 (a) A silk fabric is printed with the above paste and thereafter air-dried, heat-treated for 2 minutes at 330° F. and then soaped for 10 minutes at 140° F. in 1% soap solution. The lampblack 15 is firmly, mechanically affixed to the silk fabric, and the design is very sharp, as no bleeding occurs on soaping.

15 (b) Exactly in an analogous manner a piece of cotton fabric is printed with the above lampblack-dimethylolurea suspension with the same 20 result as above. Also here no bleeding occurs in the soaping operation.

25 (c) With the same printing paste, bleached sulphite paper sheets, or better bleached kraft paper or other suitable paper stock is printed. After air-drying, and subsequent heat-treatment on a hot plate for 2 minutes at 330° F., the pigment is very well mechanically affixed to the paper. Such printed paper may find application as an 30 improved wallpaper or for similar purposes.

**Example 8**

35 Bleached cotton yarn is impregnated with a 25% solution of dimethylolthiourea having a pH value of 4.5 (acetic acid being added to the neutral solution). The yarn is squeezed to 100% expression (double original weight), and after air-drying placed in an electric oven for 45 minutes at 126° C. Then it is dyed together with an 40 untreated sample of the same yarn, with 1% Clothfast Orange G, conc. (C.I. Sup. Pg. 35) under addition of 10% formic acid for 1/2 hour at 130° F. Then rinsed and dried. The untreated sample is dyed a very faint orange, almost white. The treated sample is dyed a deep 45 full orange shade, which color does not bleed on rinsing.

**Example 9**

50 An impregnation solution is prepared as follows:

12 gm. dimethylolurea and 3 gm. thiourea are dissolved to a total volume of 100 cc. In this solution a cotton fabric is dipped, expressed to 55 100% (double weight) and after air-drying, heat-treated on a hot plate 2 minutes at 330° F. The material is then dyed with 1% Alizarine Sapphire Blue GS (on the weight of the fabric), in presence of 10% formic acid for 45 minutes at 130° F., rinsed and dried. A very deep shade of blue is obtained, much deeper than with the use of dimethylolurea alone and of course still deeper in comparison with material not treated with carbamide-formaldehyde compounds.

**Example 10**

On a green vat dyed cotton fabric there is printed a design with the following paste:

|                    | Grams |
|--------------------|-------|
| 70 Titaniumdioxide | 30    |
| Dimethylolurea     | 25    |
| Water              | 25    |
| British gum        | 20    |
| Total              | 100   |

The fabric is then air-dried and heat-treated 2 minutes at 330° F. Then it is soaped in a 1/2% soap solution for 10 minutes at 140° F. The result is a splendid fixation of the white pigment on the green background. No noticeable loss of pigment 5 occurs during the soaping.

**Example 11**

Four samples of cotton fabric are dyed for 45 minutes at boiling temperature with 1% of Direct 10 Violet 3R (CIBA) in presence of 10% common salt, both amounts calculated on the weight of the fabric. Then the samples are rinsed and dried and the resultant color is a deep bluish red. (Sample a.)

15 Three samples are now immersed in a bath of 15% dimethylolurea and expressed to 100% (twice the original weight). The color bleeds very badly on this operation, and after air-drying the color of the samples is a medium bluish red. 20 (Sample b.)

25 The two remaining samples are now heat-treated for 2 minutes at 330° F. and the resultant color (sample c) is a somewhat deeper bluish red than sample b.

25 The last sample is now soaped for 10 minutes in a 1/2% soap solution at 140° F., then rinsed and dried. (Sample d.) No bleeding occurs during the soaping operation, and the shade of the finished sample is in strength like sample c.

30 Direct Violet 3R which is used in this experiment, is notoriously poor to washing and to be an exceptionally bad bleeding dyestuff if used on cotton. It will be noted, that the dyestuff, remaining in the fabric in this experiment, becomes not only fast to washing, but also to soap ing, after the impregnation with dimethylolurea and subsequent heat-treatment.

**Example 12**

40 Four printing pastes are prepared as follows:

(a) 15 gm. dimethylolurea, 45 gm. water, 40 gm. British gum. No further additions. Total 100 gm.

(b) 15 gm. dimethylolurea, 42 gm. water, 39.7 gm. British gum, 3.3 gm. ethylamine of 33% strength. Total 100 gm.

(c) 15 gm. dimethylolurea, 39.7 gm. water, 40 gm. British gum, 1 gm. methylamine in form of the acetate (Prepared by over-neutralizing 3.3 50 gm. (33%) methylamine solution with acetic acid to a pH=5.0.) Total 100 gm.

(d) 15 gm. dimethylolurea, 39.7 gm. water, 40 gm. British gum, 1 gm. ethylamine in form of hexamethylenetetra-ethylamine. (Prepared by adding the corresponding amount of formaldehyde to 3.3 gm. (33%) solution of ethylamine.) Total 100 gm.

With each of these pastes a cotton cloth sample is printed, air-dried and heat-treated 2 minutes at 330° F. Then the samples, weighing 4 gm. each, are dyed separately but in the same manner 60 10 cc. of 1/4% Alizarine Sapphire Blue GS (0.62% calculated on the weight of the fabric) and 1 cc. formic acid for 1/2 hour at 130° F. After 65 soaping for 10 minutes at 140° F. in 1/2% soap solution, rinsing and drying, the following results are obtained.

In all samples the untreated base is dyed a very faint blue, and in all samples the printed 70 design is dyed a much darker blue shade. The strength of the blue is deepest in experiments c and d. The strength of b is somewhat lighter, and the strength of a is again somewhat lighter than b. It appears, therefore, that the used 75

amines or amine compounds are acting as intensifiers.

*Example 13*

Bleached cotton cloth is impregnated with a 25% solution of a urea-thiourea-formaldehyde product. (Prepared by reacting 85% dimethylolurea and 15% dimethylolthiourea in the same amount of water for a long time at 100° C., until a sample of the solution, when diluted with 10 three volumes water, produces a turbidity.) The solution is then diluted to 25% with water. The cloth is then expressed to 100% (double original weight) air-dried and heat-treated on a hot plate for 2 minutes at 330° F. The fabric is then dyed with 1% Clothfast Orange G, conc. (CIBA), (Calc. on weight of sample) and 10% formic acid for 1/2 hour at 130° F. The result is a medium strength of orange, much deeper than is obtained without impregnation.

*Example 14*

A sample of linen fabric is impregnated with a 25% solution, containing 20% dimethylolurea and 5% dimethylolthiourea dissolved in water. The fabric is then air-dried and heat-treated 25 minutes at 330° F. on a hot plate. The linen sample is now dyed, simultaneously with an un-impregnated sample with 1% Clothfast Orange G, conc. (CIBA) and 10% formic acid, (calc. on the weight of the sample) for 45 minutes at 30 130° F., then rinsed and dried.—The impregnated linen dyes a very deep, full shade orange, while the untreated linen sample is practically 35 undyed and shows only a very faint tint.

*Example 15*

Solutions of formaldehyde products of urea homologues and urea derivatives are prepared as follows:

(a) 30 gm. of guanidine carbonate are reacted 40 under reflux in a boiling water bath with 60 gm. (37% vol.) formaldehyde solution for 5-10 minutes, and then cooled. The clear solution is then diluted with water to a total volume of 213 cc. (about 25% strength).

(b) 84 gm. of dicyan-diamide and 243 cc. of 45 formaldehyde (37% vol.) are reacted at 100° C. for about 10 minutes. The clear solution is then diluted to about 25% strength by bringing the 50 total volume with water to 700 cc.

(c) 300 gm. urea are heated to 160-170° C. for 12 hours, until the foaming, caused by escaping 55 ammonia has almost ceased. 18.5 gm. of the white residue is reacted with 47.3 cc. of formaldehyde (37% vol.) for about 15 minutes and the slightly turbid solution is filtered and diluted with water to about 25% strength by bringing the total volume to 148 cc.

(d) A 25% solution of carbamide-formaldehyde 60 products is prepared by dissolving 20 gm. dimethylolurea in 60 cc. water and adding thereto 20 cc. of the guanidine formaldehyde product solution as described in this example under a.

(e) A 25% solution of carbamide-formaldehyde 65 products is prepared by dissolving 20 gm. dimethylolurea in 60 cc. water and adding thereto 20 cc. of the solution b in this example, containing 5 gm. of the dicyan-diamide formaldehyde compound.

(f) A 25% solution of carbamide-formaldehyde 70 products is prepared by dissolving 20 gm. of dimethylolurea in 60 cc. water and adding thereto 20 cc. of the solution c in this example, containing 5 gm. of the formaldehyde products made of heat-treated urea.

Cotton fabrics samples are immersed in the above solutions and after expression to the double original weight, heat-treated on a hot plate for 2 minutes at 330° F. Then they are soaped for 5 minutes at 95° C. in a 1/4% soap solution, rinsed and dried.

The samples A—F impregnated with the solutions a—f respectively, are now dyed separately but under the same conditions with 1% Benzyl-green B conc. (CIBA), (Color Index 667) calc. on the weight of the samples, and 10% formic acid at 130° F. for 30 minutes.

*Results*

Sample A is dyed a medium deep green.

Sample B is dyed a full deep green.

Sample C is dyed a full deep green of a somewhat bluer tone than B.

Sample D is dyed a medium green similar to A.

Sample E is dyed a full deep green similar to C.

Sample F is dyed a light shade of green, but is still very much deeper colored than an untreated sample under the same conditions which produces only a very faint green tint.

The foregoing description and examples, it is 25 understood, are merely illustrative of the invention and in nowise limiting, as the invention includes all modifications fairly within the scope of the appended claims.

The invention is not limited to the particular 30 substances, quantities, temperatures or mode of procedure, as described, all or any of which may be varied without going beyond the scope of the invention as described and claimed.

We claim:

1. A dye fixing agent comprising a heat-treated formaldehyde condensation product of the mixture obtained by the heat treatment of urea and comprising urea, biuret, cyanuric acid and guanidine.

2. A printing mixture for cellulosic materials comprising a wool or silk dye and the initial condensation products of formaldehyde with a mixture obtained by the heat treatment of urea and comprising urea, biuret, cyanuric acid and 45 guanidine.

3. A dye fixing agent comprising a heat-treated compound obtained from the condensation of formaldehyde with a mixture of substances produced by subjecting urea to partial thermal 50 decomposition at a temperature of about 160° C.

4. A process for dyeing cotton, rayon or other fibrous materials with a wool or silk dye comprising affixing the dye by a heat treatment of the fibrous material in presence of the products obtained by the reaction between formaldehyde and the products of the partial thermal decomposition of urea at a temperature of about 160° C.

5. A colored fibrous cellulosic material wherein 60 a wool or silk dye is chemically affixed with a heat-treated substance resulting from the condensation of formaldehyde with a mixture comprising biuret, cyanuric acid, guanidine and urea and obtained by subjecting urea to a heat-treatment at a temperature of about 160° C.

6. A dyeing mixture for cellulosic materials comprising a wool or silk dye and the initial condensation products of formaldehyde with a mixture of substances obtained by subjecting urea to a heat treatment at a temperature of about 160° C.

7. A process for dyeing cotton, rayon or other vegetable fibers with wool or silk dyes, comprising chemically affixing the wool or silk dye with the initial condensation products of formaldehyde with preliminarily heat-treated urea.

8. A process for dyeing cotton, rayon or other vegetable fibers with wool or silk dyes, comprising treating the fibrous material with the initial condensation products of formaldehyde with preliminarily heat-treated urea, then subjecting the resultant fibrous material to a heat treatment, and finally dyeing the heat-treated fibrous material with a wool or silk dye. 5
9. A process for dyeing cotton, rayon or other vegetable fibers with wool or silk dyes, comprising 10 treating the fibrous material with the initial condensation products of formaldehyde with the mixture obtained by subjecting urea to a thermal treatment at a temperature of about 160° C., thereafter subjecting the fibrous material to heat treatment, and then dyeing it with a wool or silk dye. 15
10. A dyeing mixture for cellulosic materials comprising a wool or silk dye and the initial condensation products of formaldehyde with preliminarily heat-treated and partially thermally 20 decomposed urea.
11. A colored cellulosic material wherein the wool or silk dye is chemically affixed with the initial condensation products of formaldehyde with preliminarily heat-treated and partially thermally 5 decomposed urea.
12. A process for dyeing cotton, rayon or other fibrous materials with a wool or silk dye comprising affixing the dye used by a heat treatment of the fibrous material in presence of a formaldehyde compound of heat-treated and partially thermally 10 decomposed urea.
13. A colored fibrous material wherein the coloring matter is mechanically affixed with a heat-treated formaldehyde compound of heat-treated urea. 15
14. A colored fibrous cellulosic material wherein a wool or silk dye is chemically affixed with a heat-treated formaldehyde compound of heat-treated urea. 20

GUSTAVE A. WIDMER.

EDWARD W. PIERCE.